

UNITED STATES PATENT OFFICE

2,217,009

## PROCESS OF CONVERTING ACETYLENIC HYDROCARBONS TO AROMATIC HYDROCARBONS

**Aristid V. Grosse and William J. Mattox, Chicago,  
Ill., assignors to Universal Oil Products Com-  
pany, Chicago, Ill., a corporation of Delaware**

No Drawing. Application May 31, 1938,  
Serial No. 211,018

**6 Claims. (Cl. 260—668)**

This invention relates more particularly to the conversion of straight chain hydrocarbons into closed chain cyclic hydrocarbons.

conditions of operation by the present types of catalysts, the following structural equations are introduced:

More specifically it is concerned with a process involving the use of special catalysts and specific conditions of operation in regard to temperature, pressure, and time of reaction whereby certain types of acetylenic hydrocarbons can be efficiently converted into aromatic hydrocarbons.

10 The search for catalysts to specifically control and accelerate desired conversion reactions among hydrocarbons has been attended with the usual difficulties encountered in finding catalysts for other types of reactions since there are no  
15 basic laws or rules for predicting the effectiveness of catalytic materials and the art as a whole is in a more or less empirical state. In using many catalysts even in connection with conversion reactions among pure hydrocarbons

and particularly in connection with the conversion of the relatively heavy distillates and residua which are available for cracking, there is a general tendency for the decomposition reactions to proceed at a very rapid rate, necessitating the use of extremely short time factors and very accurate control of temperature and pressure to avoid too extensive decomposition. There are further difficulties encountered in maintaining the efficiency of catalysts employed in pyrolysis since there is usually a rapid deposition of carbonaceous materials on their surfaces and in their pores.

In one specific embodiment the present invention comprises the conversion of acetylenic hydrocarbons having six or more carbon atoms in straight chain arrangement into aromatic hydrocarbons by subjecting them at elevated temperatures of the order of 450-700° C. to contact for definite times of the order of 0.1-30 seconds with catalytic materials comprising major proportions of refractory carriers of relatively low catalytic activity supporting minor proportions of compounds of elements selected from those occurring in the lefthand column of Group IV of the periodic table, these compounds having relatively high catalytic activity.

In accordance with the present invention, acetylenic hydrocarbons such as hexine, heptine, and octine are dehydrogenated and cycled in such a way that the chains of carbon atoms undergo ring closure to produce benzene or higher molecular weight alkyl derivatives thereof. For the sake of illustrating and exemplifying the type of hydrocarbon conversion reactions which are accelerated under the preferred



Under properly controlled conditions of times of contact, temperature, and pressure which obviously vary with the particular compound undergoing treatment, once-through yields of aromatics of the order of 25% to 50% by weight are obtainable which can be increased to over 70% by recycling the unconverted material. This type of reaction was unpredictable in view of the type of hydrocarbon furnishing the starting material and the results obtained were quite unexpected. The reaction mechanisms leading to the formation of aromatics from the acetylenic hydrocarbons are probably of a complicated character since there must obviously be some shifting of the bonds between carbon atoms to produce aromatics characterized by so-called alternate double bonds.

It will be seen from the foregoing that the scope of the present invention is preferably limited to the treatment of acetylenic hydrocarbons which contain at least 6 carbon atoms in straight chain arrangement. In the case of acetylene hydrocarbons containing less than 6 carbon atoms in linear arrangement, some formation of aromatics may take place due to primary isomerization and/or polymerization reactions although obviously the extent of these will vary considerably with the type of compound and the conditions of operation. The process is readily applicable to acetylenes from hexene up

to dodecene. With increase in molecular weight beyond this point the percentage of undesirable side reactions tends to increase and yields of the desired alkylated aromatics decrease in proportion.

The present invention is characterized by the use of a particular group of composite catalytic materials which employ as their base catalysts certain refractory oxides and silicates which in themselves may have some slight specific catalytic ability in the dehydrogenation and cyclization reactions but which are improved greatly in this respect by the addition of certain promoters or secondary catalysts in minor proportions. These base supporting materials are preferably of a rugged and refractory character capable of withstanding the severe use to which the catalysts are put in regard to temperature during service and in regeneration by means of air or other oxidizing gas mixtures after they have become fouled with carbonaceous deposits after a period of service. As examples of materials which may be employed in granular or pelleted form as supports for the preferred catalytic substances may be mentioned the following:

|                 |                        |
|-----------------|------------------------|
| Magnesium oxide | Montmorillonite clays  |
| Aluminum oxide  | Kieselguhr             |
| Bauxite         | Crushed firebrick      |
| Bentonite clays | Crushed silica         |
|                 | Glauconite (greensand) |

It should be emphasized that in the field of catalysis there have been very few rules evolved which will enable the prediction of what materials will catalyze a given reaction. Most of the catalytic work has been done on a purely empirical basis, even though at times certain groups of elements or compounds have been found to be more or less equivalent in accelerating certain types of reactions.

In regard to the base catalytic materials which are preferably employed according to the present invention, some precautions are necessary to insure that they possess proper physical and chemical characteristics before they are impregnated with the promoters to render them more efficient. In regard to magnesium oxide, which may be alternatively employed, this is most conveniently prepared by the calcination of the mineral magnesite which is most commonly encountered in a massive or earthy variety and rarely in crystal form, the crystals being usually rhombohedral. In many natural magnesites, the magnesium oxide may be replaced to the extent of several per cent by iron oxide. The mineral is of quite common occurrence and readily obtainable in quantity at a reasonable figure. The pure compound begins to decompose to form the oxide at a temperature of 350° C., though the rate of decomposition only reaches a practical value at considerably higher temperatures, usually of the order of 800° C. to 900° C. Magnesite is related to dolomite, the mixed carbonate of calcium and magnesium, which latter mineral, however, is not of as good service as the relatively pure magnesite in the present instance. Magnesium carbonate prepared by precipitation or other chemical methods may be used alternatively in place of the natural mineral. It is not necessary that the magnesite be completely converted to oxide but as a rule it is preferable that the conversion be at least over 90%, that is, so that there is less than 10% of the original carbonate remaining in the ignited material.

75 Aluminum oxide which is generally preferable

as a base material for the manufacture of catalysts for the process may be obtained from natural aluminum oxide minerals or ores such as bauxite or carbonates such as dawsonite by proper calcination, or it may be prepared by precipitation of aluminum hydrate from solutions of aluminum sulfate, nitrate, chloride, or different other salts, such as alums, and dehydration of the precipitate of aluminum hydroxide by heat. Usually it is desirable and advantageous to further treat it with air or other gases, or by other means to activate it prior to use.

Three hydrated oxides of aluminum occur in nature, to wit, hydrargillite or gibbsite having the formula  $Al_2O_3 \cdot 3H_2O$ , bauxite having the formula  $Al_2O_3 \cdot 2H_2O$ , and diasporite having the formula  $Al_2O_3 \cdot H_2O$ . Of these three minerals the corresponding oxides from the trihydrated and dihydrated minerals are suitable for the manufacture of the present type of catalysts and these materials have furnished types of activated alumina which are entirely satisfactory as supports for the preferred catalysts. Precipitated trihydrates can also be dehydrated at moderately elevated temperatures to form satisfactory alumina supports. The mineral dawsonite having the formula  $Na_3Al(CO_3)_3 \cdot 2Al(OH)_3$  is another mineral which may be used as a source of aluminum oxide, the calcination of this mineral giving an alkalinized aluminum oxide which is apparently more effective as a support in that the catalyst is more easily regenerated after a period of service. Alumina in the form of powdered corundum is not suitable as a base.

It is best practice in the final steps of preparing aluminum oxide as a base catalyst to ignite the hydrated oxides for some time at temperatures within the approximate range of 600-750° C., which probably does not correspond to complete dehydration of the hydroxides but apparently gives a catalytic material of good strength and porosity so that it is able to resist for a long period of time the deteriorating effects of the service and regeneration periods to which it is subjected. In the case of the clays which may serve as base catalytic material for supporting promoters, the better materials are those which have been acid treated to render them more siliceous. These may be pelleted or formed in any manner before or after the addition of the promoter catalyst since ordinarily they have a high percentage of fines. The addition of certain of the promoters, however, exerts a binding influence so that the formed materials may be employed without fear of structural deterioration in service.

Our investigations have also definitely demonstrated that the catalytic efficiency of such substances as alumina, magnesium oxide, and clays which may have some catalytic potency in themselves is greatly improved by the presence of compounds of the preferred elements in relatively minor amounts, usually of the order of less than 10% by weight of the carrier. It is most common practice to utilize catalysts comprising 2 to 5% by weight of these compounds, particularly their lower oxides.

The promoters which are used in accordance with the present invention to produce active catalysts of the base materials include generally compounds and more particularly oxides of the elements in the lefthand column of Group IV of the periodic table including titanium, zirconium, cerium, hafnium, and thorium. In general practically all of the compounds of the preferred

elements will have some catalytic activity though as a rule the oxides and particularly the lower oxides are the best catalysts. Catalyst composites may be prepared by utilizing the soluble compounds of the elements in aqueous solutions, from which they are absorbed by prepared granular carriers or from which they are deposited upon the carriers by evaporation of the solvent. The invention further comprises the use of catalyst composites made by mixing relatively insoluble compounds with carriers either in the wet or the dry condition. In the following paragraphs some of the compounds of the elements listed above are given which are soluble in water and which may be used to add catalytic material to carriers. The known oxides of these elements are also listed.

### Titanium

Compounds which will ultimately yield titanium catalysts on heating to a proper temperature are absorbed by stirring them with warm aqueous solutions of soluble titanium compounds, such as for example titanium nitrate having the formula  $5\text{TiO}_2\text{N}_2\text{O}_5\cdot 6\text{H}_2\text{O}$ , which is sufficiently soluble in warm water to render it readily utilizable as a source of titanium oxides. Other soluble compounds which may be used to form catalytic deposits containing titanium are the various alkali metal titanates. Other compounds of titanium acids, including compounds of the alkaline earth and heavy metals may be distributed upon the carriers by mechanical mixing either in the wet or the dry condition. The lower oxides are generally the best catalysts. The oxide resulting from the decomposition of such compounds as the nitrate and the hexahydrate is for the most part the dioxide  $\text{TiO}_2$ . This oxide, however, is reduced by hydrogen, or by the gases and vaporous products resulting from the decomposition of the mono-olefins treated in the first stages of the reactions so that the essential catalyst for the larger portion of the period of service is the sesquioxide  $\text{Ti}_2\text{O}_3$ .

### Zirconium

The soluble compounds of zirconium which may be used as primary sources of catalytic materials in aqueous solution include the slightly soluble zirconium ammonium fluoride, the tetrachloride, the fluoride, the iodide and particularly the more soluble selenate and sulfate. The crystalline selenate has the formula  $\text{Zr}(\text{SeO}_4) \cdot 2\text{H}_2\text{O}$  and the sulfate which is the more soluble of the two, has the formula  $\text{Zr}(\text{SO}_4) \cdot 2\text{H}_2\text{O}$ . As in the case of the other alternative elements the tetrahydroxide may be precipitated from a solution of the sulfate or other soluble salt onto the surface and into the pores of an active granular carrier by the addition of alkaline carbonate or hydroxide precipitants, after which the zirconium hydroxide is ignited to produce the dioxide. The principal oxide of zirconium is the dioxide and there is little evidence to indicate the existence of a monoxide since the dioxide is not reducible by hydrogen at moderate temperatures and it has been shown that carbon in the electric furnace reduces the dioxide directly to the metal.

### Cerium

A properly prepared and activated carrier is ground and sized to produce granules of relatively small mesh of the approximate order of from 4 to 20 and these may be caused to absorb compounds which will ultimately yield compounds

of cerium on heating to a proper temperature by stirring them with warm aqueous solutions of soluble cerium compounds, such, as for example cerium nitrate having the formula  $\text{Ce}(\text{NO}_3)_3 \cdot 6\text{H}_2\text{O}$ , which is sufficiently soluble in warm water to render it readily utilizable as a source of cerium oxides. Other soluble compounds which may be used to form catalytic deposits containing cerium are the various alkali metal cerous nitrates, such as for example sodium cerous nitrate having the formula  $2\text{NaNO}_3 \cdot \text{Ce}(\text{NO}_3)_3 \cdot \text{H}_2\text{O}$ . As a rule the lower oxides are the best catalysts. Cerium has a number of oxides including the trioxide  $\text{CeO}_3$ , the dioxide  $\text{CeO}_2$ , the heptoxide  $\text{Ce}_4\text{O}_7$ , and sesquioxide  $\text{Ce}_2\text{O}_3$ . The dioxide results from the ignition of cerous nitrate, cerous sulfate, cerous carbonate or cerous oxalate and also from the ignition of ceric nitrate, ceric sulfate or ceric hydroxide. Hydrogen reduces the dioxide to the heptoxide, and it is probable that this oxide plus a certain amount of the sesquioxide are active catalysts.

### Hafnium

In general the properties of hafnium from a chemical and to some extent a catalytic standpoint are intermediate between those of zirconium and thorium though in most reactions hafnium compounds more closely correspond to those of zirconium. There is but one known oxide, the dioxide  $\text{HfO}_2$  and this oxide is not readily reducible and probably exists as such when used in minor proportions as a constituent of catalyst composites in hydrocarbon dehydrogenation reactions. Soluble compounds of hafnium include the oxychloride having the formula  $\text{HfOCl}_2 \cdot 8\text{H}_2\text{O}$  and the oxalate which is soluble in an excess of oxalic acid. The mixing of this oxalate solution with the miscellaneous carriers proposed and the evaporation of the solution gives a residual material which can be ignited to leave a residue of the dioxide. Hafnium sulfate catalysts may be developed by igniting composites of relatively inert carriers and hafnium sulfate at temperatures of about  $500^{\circ}\text{C}$ . On account of the rarity of hafnium its compounds are seldom commercially utilizable although the oxide in particular has been found to exert a good catalytic influence in the types of reactions under consideration.

### Thorium

The element thorium furnishes a number of compounds which can be used as primary sources of catalytic material for deposition upon the types of carriers disclosed. The following compounds are sufficiently soluble in water to enable them to be used in aqueous solution to saturate prepared granular carrier particles: the bromide  $\text{ThBr}_4$ , the chloride  $\text{ThCl}_4$ , the iodide  $\text{ThI}_4$ , and the nitrate  $\text{Th}(\text{NO}_3)_4$  which is most conveniently used as the tetrahydrated or dodecahydrated salt. From any of the soluble salts mentioned the tetrahydroxide  $\text{Th}(\text{OH})_4$  may be precipitated by the use of alkali carbonates or alkali hydroxides and then ignited to produce the dioxide. The phosphates and sulfates and the sulfide are relatively insoluble and may be incorporated with the carrier particles either in the wet or the dry condition. The nitrate may be directly ignited, of course, to produce the dioxide.

While the identification of some other oxides of thorium such as the pentatrioxide  $\text{Th}_3\text{O}_5$  and

the monoxide  $\text{ThO}$  has been claimed as well as a peroxide having the formula  $\text{Th}_2\text{O}_7$ , it has been shown that the principal oxide catalyst in operations of the present character is the ordinary dioxide. It is to be emphasized that the oxide is the preferred catalyst since in general it exhibits greater and more selective catalytic action than any other compounds which may be formed upon the carrier surfaces.

10 The most general method for adding promoting materials to the preferred base catalysts, which if properly prepared have a high adsorptive capacity, is to stir the prepared granules of from approximately 4 to 20 mesh into solutions 15 of salts which will yield the desired promoting compounds on ignition under suitable conditions. In some instances the granules may be merely stirred in slightly warm solutions of salts until the dissolved compounds have been retained on 20 the particles by absorption or occlusion, after which the particles are separated from the excess solvent by settling or filtration, washed with water to remove excess solution, and then ignited to produce the desired residual promoter.

25 In cases of certain compounds of relatively low solubility it may be necessary to add the solution in successive portions to the adsorbent base catalyst with intermediate heating to drive off solvent in order to get the required quantity of 30 promoter deposited upon the surface and in the pores of the base catalyst. The temperatures used for drying and calcining after the addition of the promoters from solutions will depend entirely upon the individual characteristics of the 35 compound added and so general ranges of temperature can be given for this step.

In some instances promoters may be deposited from solution by the addition of precipitants which cause the deposition of precipitates upon 40 the catalyst granules. As a rule methods of mechanical mixing are not preferable, though in some instances in the case of hydrated or readily fusible compounds these may be mixed with the proper proportions of base catalysts and uniformly distributed during the condition of fusing or fluxing.

In regard to the relative proportions of base catalyst and promoting materials it may be stated in general that the latter are less than 50 10% by weight of the total composites. The effect upon the catalytic activity of the base catalysts caused by varying the percentage of any given compound or mixture of compounds deposited thereon is not a matter for exact calculation but more one for determination by experiment. Frequently good increases in catalytic effectiveness are obtainable by the deposition of as low as 1% or 2% of a promoting compound upon the surface and in the pores of the base 55 catalyst, though the general average is about 5%.

It has been found essential to the production of high yields of aromatics from acetylenic hydrocarbons when using the preferred types of catalysts that depending upon the acetylenic hydrocarbons or mixture of hydrocarbons being treated, temperatures from 450-700° C. should be employed, contact times of approximately 60 0.1 to 30 seconds and pressures approximating atmospheric. The times of contact most commonly employed with acetylenic hydrocarbons having from 6-12 carbon atoms to the molecule are of the order of 10 to 20 seconds. It will be appreciated by those familiar with the art of hydrocarbon conversion in the presence of catalysts that the factors of temperature, pressure,

and time will frequently have to be adjusted from the results of preliminary experiments to produce the best results in any given instance. The criterion of the yield of an aromatic having the same number of carbon atoms in the ring as the original acetylenic hydrocarbon charged had in the chain will serve to fix the best conditions of operation. In a general sense, the relations between time, temperature, and pressure are preferably adjusted so that rather intensive 10 conditions are employed of sufficient severity to insure a maximum amount of the desired cyclization reactions with a minimum of undesirable side reactions.

In operating the process the general procedure is to vaporize hydrocarbons or mixtures of hydrocarbons and after heating the vapors to a suitable temperature within the ranges previously specified, to pass them through stationary masses of granular catalytic material in vertical cylindrical treating columns or banks of catalyst-containing tubes in parallel connection. Since the reactions are endothermic it may be necessary to apply some heat externally to maintain the best reaction temperature. After passing through the catalytic zone the products are submitted to fractionation to recover cuts or fractions containing the desired aromatic product with the separation of fixed gases, unconverted hydrocarbons and heavier residual materials, which may be disposed of in any suitable manner depending upon their composition. The overall yield of aromatics may be increased by recycling the unconverted acetylenic hydrocarbons to further treatment with fresh material, although this is 35 a more or less obvious expedient and not specifically characteristic of the present invention.

The present types of catalysts owing to their more or less specific action under the limited conditions of operation specified maintain their 40 activity over relatively long periods of time. However, when their activity begins to diminish after a period of service, it is readily regenerated by the simple expedient of oxidizing with air or other oxidizing gas at a moderately elevated temperature, usually within the range employed in the dehydrogenation and cyclization reactions. This oxidation effectively removes traces of carbon deposits which contaminate the surface of the particles and decrease their efficiency. It is 50 characteristic of the present types of catalysts that they may be repeatedly regenerated with only a very gradual loss of catalytic efficiency.

During oxidation with air or other oxidizing gas mixture in regenerating partly spent material, there is evidence to indicate that when the lower oxides are employed, they are to a large extent, if not completely, oxidized to higher oxides which combine with basic carriers to form compounds of variable composition. Later these compounds are decomposed by contact with reducing gases in the first stages of service to reform the lower oxides and regenerate the real catalyst and hence the catalytic activity.

#### Example I

The general procedure for manufacturing the catalyst was to dissolve titanium nitrate in cold water and utilize this solution as a means of eventually adding titanium oxides to a carrier. 70 A saturated solution of titanium nitrate in 100 parts of water was prepared and the solution was then added to about 250 parts by weight of activated alumina which had been produced by calcining bauxite at a temperature of about 700° C., 75

followed by grinding and sizing to produce particles of approximately 8-12 mesh. Using the proportions stated, the alumina exactly absorbed the solution and the particles were first dried at 5 100° C. for about two hours and the temperature was then raised to 350° C. in a period of eight hours. After this calcining treatment the particles were placed in a reaction chamber and the titanium oxides reduced in a current of hydrogen 10 at about 500° C., when they were then ready for service.

Hexine-1 was vaporized and passed over the granular catalyst prepared as described, using a temperature of 510° C., substantially atmospheric 15 pressure, and a time of contact of 16 seconds. The yield of pure benzene under these conditions was found to be 24 by weight of the normal hexine-1 charged. By recycling of the unconverted material the ultimate yield of benzene was 20 raised to 55%.

*Example II*

Heptine-1 was treated with the same type of catalyst as in Example I at a temperature of 530° 25 C., substantially atmospheric pressure and 12 seconds contact time. The yield of toluene on a once-through basis was found to be 26 by weight and again it was found that by recycling the unconverted heptine-1 the yield of the desired 30 toluene could ultimately be brought to 52%.

*Example III*

To manufacture granular catalyst, particles of activated alumina prepared by calcination at a 35 temperature of about 1500° F., the particles varying in size from approximately 10 to 20 mesh, were stirred in a moderately saturated solution of zirconium sulfate while adding a solution of 40 sodium hydroxide to precipitate zirconium hydroxide on the alumina particles. Subsequent filtering and washing of the granules was followed by the ignition of the hydroxide to produce zirconium dioxide which acted as the catalyst. Hexine-1 was vaporized and passed over the 45 granular catalyst prepared as described, using a temperature of 550° C., substantially atmospheric pressure, and a time of contact of 15 seconds. The yield of pure benzene under these 50 conditions was found to be 16% by weight of the hexine-1 charged. By recycling of the unconverted material the ultimate yield of benzene was raised to 43%.

*Example IV*

55 The general procedure in the preparation of the catalyst was to dissolve cerous nitrate in water and utilize this solution as a means of adding cerium oxides to a carrier. 20 parts by weight of cerous nitrate was dissolved in about 100 parts by 60 weight of water, and the solution was then added to about 250 parts by weight of activated alumina which had been produced by calcining bauxite at a temperature of about 700° C. followed by grinding and sizing to produce particles of 8-12 mesh. 65 Using the proportions stated the alumina exactly absorbed the solution and the particles were first dried at 100° C. for about two hours and the temperature was then raised to 350° C. in a period of eight hours. After this calcining treatment the 70 particles were placed in a reaction chamber and the cerium dioxide reduced in a current of hydrogen at about 500° C. to produce the oxide Ce<sub>2</sub>O<sub>3</sub> when they were then ready for service.

Hexine-1 was vaporized and passed over the 75 granular catalyst comprising an alumina base

supporting about 4% by weight of the cerous oxide, using a temperature of 630° C., substantially atmospheric pressure, and a time of contact of 5 seconds. The yield of pure benzene under these conditions was found to be 26% by weight of the 5 hexine-1 charged. By recycling of the unconverted material the ultimate yield of benzene was raised to 72%.

We claim as our invention:

1. A process for the production of aromatic hydrocarbons from acetylene hydrocarbons having at least 6 carbon atoms in straight-chain arrangement, which comprises dehydrogenating and cyclizing the acetylene hydrocarbon by subjection to a temperature of the order of 450 to 700° 15 C. for a period of about 0.1 to 30 seconds in the presence of a compound of a metal from the left-hand column of Group IV of the periodic table and selected from the class consisting of titanium, 20 zirconium, cerium, hafnium and thorium.

2. A process for the production of aromatic hydrocarbons from acetylene hydrocarbons having at least 6 carbon atoms in straight-chain arrangement, which comprises dehydrogenating and cyclizing the acetylene hydrocarbon by subjection to a temperature of the order of 450 to 700° 25 C. for a period of about 0.1 to 30 seconds in the presence of an oxide of a metal from the left-hand column of Group IV of the periodic table and selected from the class consisting of titanium, 30 zirconium, cerium, hafnium and thorium.

3. A process for the production of aromatic hydrocarbons from acetylene hydrocarbons having at least 6 carbon atoms in straight-chain arrangement, which comprises dehydrogenating and 35 cyclizing the acetylene hydrocarbon by subjection to a temperature of the order of 450 to 700° C. for a period of about 0.1 to 30 seconds in the presence of a solid granular catalyst comprising a major proportion of a carrier of relatively 40 low catalytic activity supporting a minor proportion of a compound of a metal from the left-hand column of Group IV of the periodic table and selected from the class consisting of titanium, zirconium, cerium, hafnium and thorium. 45

4. A process for the production of aromatic hydrocarbons from acetylene hydrocarbons having at least 6 carbon atoms in straight-chain arrangement, which comprises dehydrogenating and cyclizing the acetylene hydrocarbon by subjection to a temperature of the order of 450 to 700° 50 C. for a period of about 0.1 to 30 seconds in the presence of a solid granular catalyst comprising a major proportion of a carrier of relatively 55 low catalytic activity supporting a minor proportion of an oxide of a metal from the left-hand column of Group IV of the periodic table and selected from the class consisting of titanium, zirconium, cerium, hafnium and thorium.

5. A process for the production of aromatic hydrocarbons from acetylene hydrocarbons having at least 6 carbon atoms in straight-chain arrangement, which comprises dehydrogenating and cyclizing the acetylene hydrocarbon by subjection to a temperature of the order of 450 to 700° 60 C. for a period of about 0.1 to 30 seconds in the presence of aluminum oxide supporting a relatively small amount of a compound of a metal from the left-hand column of Group IV of the 65 periodic table and selected from the class consisting of titanium, zirconium, cerium, hafnium and thorium.

6. A process for the production of aromatic hydrocarbons from acetylene hydrocarbons hav- 75

ing at least 6 carbon atoms in straight-chain arrangement, which comprises dehydrogenating and cyclizing the acetylene hydrocarbon by subjection to a temperature of the order of 450 to 5 700° C. for a period of about 0.1 to 30 seconds in the presence of aluminum oxide supporting a relatively small amount of an oxide of a metal from

the lefthand column of Group IV of the periodic table and selected from the class consisting of titanium, zirconium, cerium, hafnium and thorium.

ARISTID V. GROSSE.  
WILLIAM J. MATTOX.